



US007252694B2

(12) **United States Patent**  
**Woo et al.**

(10) **Patent No.:** **US 7,252,694 B2**  
(45) **Date of Patent:** **Aug. 7, 2007**

(54) **ABRASIVE ARTICLE AND METHODS OF  
MAKING SAME**

2,984,052 A 5/1961 Mueller, Jr.  
3,021,649 A 2/1962 Robbins  
3,353,308 A 11/1967 Zane  
3,420,007 A 1/1969 Kolesh  
3,861,892 A 1/1975 Wisdom, Jr. et al.  
3,932,966 A 1/1976 Stern  
4,001,366 A 1/1977 Brumlik  
4,062,152 A 12/1977 Mehrer  
4,158,935 A 6/1979 Robert  
4,282,011 A 8/1981 Terpay  
4,287,685 A 9/1981 Marton  
4,437,269 A 3/1984 Shaw  
4,590,113 A 5/1986 Herzog  
4,609,581 A 9/1986 Ott

(75) Inventors: **Edward J. Woo**, Woodbury, MN (US);  
**Charles R. Wald**, Oakdale, MN (US);  
**Curtis J. Schmidt**, South St. Paul, MN  
(US)

(73) Assignee: **3M Innovative Properties Company**,  
St. Paul, MN (US)

(\*) Notice: Subject to any disclaimer, the term of this  
patent is extended or adjusted under 35  
U.S.C. 154(b) by 0 days.

(21) Appl. No.: **11/198,265**

(22) Filed: **Aug. 5, 2005**

(Continued)

(65) **Prior Publication Data**

US 2007/0028526 A1 Feb. 8, 2007

FOREIGN PATENT DOCUMENTS

DE 34 16 186 A1 1/1985

(51) **Int. Cl.**

*B24D 3/00* (2006.01)  
*B24D 11/02* (2006.01)  
*B24D 18/00* (2006.01)  
*B24B 11/00* (2006.01)

(Continued)

(52) **U.S. Cl.** ..... **51/298**; 51/307; 51/308;  
51/309; 51/293; 451/526; 451/532; 451/538;  
451/539; 451/536

U.S. Appl. No. 11/321,505, Woo et al., filed Dec. 29, 2005.

(Continued)

(58) **Field of Classification Search** ..... 51/298,  
51/307-309, 293; 451/526, 532, 538, 536,  
451/539

Primary Examiner—Michael Marcheschi

See application file for complete search history.

(56) **References Cited**

U.S. PATENT DOCUMENTS

1,850,413 A 3/1932 Porte  
1,862,103 A 6/1932 Stratford  
1,961,911 A 6/1934 Pusch  
2,123,581 A 7/1938 Anderson  
2,740,239 A 4/1956 Ball et al.  
2,749,681 A 6/1956 Reidenbach  
2,838,890 A 6/1958 McIntyre

A porous abrasive article that allows air and dust particles to pass through. The abrasive article has a screen abrasive and an apertured attachment interface with hooks. The screen abrasive has an abrasive layer comprising a plurality of abrasive particles and at least one binder. The apertured attachment interface cooperates with the screen abrasive to allow the flow of particles through the abrasive article.

**20 Claims, 5 Drawing Sheets**



## U.S. PATENT DOCUMENTS

|                 |         |                             |
|-----------------|---------|-----------------------------|
| 4,631,220 A     | 12/1986 | Clifton                     |
| 4,645,699 A     | 2/1987  | Neveu                       |
| 4,722,203 A     | 2/1988  | Darjee                      |
| 4,725,487 A     | 2/1988  | Pemrick et al.              |
| 4,759,155 A     | 7/1988  | Shaw                        |
| 4,844,967 A     | 7/1989  | Goralski et al.             |
| 4,920,702 A     | 5/1990  | Kloss et al.                |
| 4,932,163 A     | 6/1990  | Chilton et al.              |
| 4,937,984 A     | 7/1990  | Taranto                     |
| 4,964,243 A     | 10/1990 | Reiter                      |
| 4,964,245 A     | 10/1990 | Braasch                     |
| 5,007,206 A     | 4/1991  | Paterson                    |
| 5,036,627 A     | 8/1991  | Walters                     |
| 5,131,924 A     | 7/1992  | Wiand                       |
| 5,254,194 A     | 10/1993 | Ott et al.                  |
| 5,256,231 A     | 10/1993 | Gorman et al.               |
| 5,317,886 A     | 6/1994  | Prahl                       |
| 5,354,591 A     | 10/1994 | Ott et al.                  |
| 5,367,839 A     | 11/1994 | Pearce                      |
| 5,389,032 A     | 2/1995  | Beardsley                   |
| 5,458,532 A     | 10/1995 | Cannone                     |
| 5,490,878 A     | 2/1996  | Peterson et al.             |
| 5,505,747 A     | 4/1996  | Chesley et al.              |
| 5,533,923 A     | 7/1996  | Shamoulian et al.           |
| 5,578,343 A *   | 11/1996 | Gaeta et al. .... 427/202   |
| 5,607,345 A     | 3/1997  | Barry et al.                |
| 5,616,394 A     | 4/1997  | Gorman et al.               |
| 5,667,540 A     | 9/1997  | Chesley et al.              |
| 5,674,122 A *   | 10/1997 | Krech .... 451/536          |
| 5,695,533 A     | 12/1997 | Kardys et al.               |
| 5,807,161 A     | 9/1998  | Manor et al.                |
| 5,810,650 A     | 9/1998  | Jöst                        |
| 5,891,549 A     | 4/1999  | Beretta et al.              |
| 5,904,793 A     | 5/1999  | Gorman et al.               |
| 5,954,844 A     | 9/1999  | Law et al.                  |
| 5,989,112 A     | 11/1999 | Long et al.                 |
| 6,024,634 A *   | 2/2000  | Hoglund et al. .... 451/532 |
| 6,059,644 A     | 5/2000  | Manor et al.                |
| 6,074,292 A     | 6/2000  | Gilday                      |
| 6,077,156 A     | 6/2000  | Amin et al.                 |
| 6,077,601 A     | 6/2000  | DeVoe et al.                |
| 6,190,246 B1    | 2/2001  | Parrott et al.              |
| 6,197,076 B1    | 3/2001  | Braunschweig et al.         |
| 6,280,824 B1    | 8/2001  | Insley et al.               |
| 6,312,325 B1    | 11/2001 | Van Osenbruggen             |
| 6,368,199 B1    | 4/2002  | Van Osenbruggen             |
| 6,482,308 B1    | 11/2002 | Wiemann                     |
| 6,575,821 B2    | 6/2003  | Jöst                        |
| 6,579,162 B2    | 6/2003  | Chesley et al.              |
| 6,613,113 B2    | 9/2003  | Minick et al.               |
| 6,790,126 B2    | 9/2004  | Wood et al.                 |
| 6,923,840 B2    | 8/2005  | Schutz et al.               |
| 2003/0003856 A1 | 1/2003  | Swei                        |
| 2003/0127108 A1 | 7/2003  | Policicchio et al.          |
| 2003/0143938 A1 | 7/2003  | Braunschweig et al.         |
| 2003/0159363 A1 | 8/2003  | Chesley et al.              |
| 2004/0098923 A1 | 5/2004  | Hood et al.                 |
| 2004/0109978 A1 | 6/2004  | Michel                      |
| 2004/0148866 A1 | 8/2004  | Krupnick                    |

|                  |         |                          |
|------------------|---------|--------------------------|
| 2004/0166788 A1  | 8/2004  | Travis                   |
| 2004/0170801 A1* | 9/2004  | Seth et al. .... 428/100 |
| 2004/0170802 A1* | 9/2004  | Seth et al. .... 428/100 |
| 2004/0209561 A1  | 10/2004 | Suzuki et al.            |
| 2005/0124274 A1  | 6/2005  | Hoglund                  |
| 2006/0019579 A1  | 1/2006  | Braunschweig             |

## FOREIGN PATENT DOCUMENTS

|    |                 |         |
|----|-----------------|---------|
| DE | 41 24 520 A1    | 1/1993  |
| DE | 201 11 245 U 1  | 8/2001  |
| EP | 0 064 748       | 8/1984  |
| EP | 0 166 060       | 9/1988  |
| EP | 0 285 042 A1    | 10/1988 |
| EP | 0 578 865 A1    | 1/1994  |
| EP | 0 738 562       | 10/1996 |
| EP | 1 488 888 A1    | 12/2004 |
| EP | 1 524 077 A1    | 4/2005  |
| EP | 1 733 844 A1    | 12/2006 |
| FR | 2 659 892       | 9/1991  |
| FR | 2 739 308       | 4/1997  |
| GB | 1137556         | 12/1968 |
| GB | 1539477         | 1/1970  |
| GB | 2 017 485 A     | 10/1979 |
| GB | 2 057 483 A     | 4/1981  |
| GB | 2 162 213 A     | 1/1986  |
| GB | 2 199 053 A     | 6/1988  |
| JP | 5-220670        | 8/1993  |
| JP | 11-179668       | 7/1999  |
| WO | WO 90/14039     | 11/1990 |
| WO | WO 96/07509     | 3/1996  |
| WO | WO 00/46434     | 11/2000 |
| WO | WO 03/020474 A1 | 3/2003  |

## OTHER PUBLICATIONS

|                                                                                                                                                                                                                                                                                                                  |
|------------------------------------------------------------------------------------------------------------------------------------------------------------------------------------------------------------------------------------------------------------------------------------------------------------------|
| U.S. Appl. No. 11/197,798, Woo et al., filed Aug. 5, 2005.                                                                                                                                                                                                                                                       |
| U.S. Appl. No. 11/228,896, Rambosek et al., filed Sep. 16, 2005.                                                                                                                                                                                                                                                 |
| U.S. Appl. No. 11/229,277, Woo et al., filed Sep. 16, 2005.                                                                                                                                                                                                                                                      |
| U.S. Appl. No. 11/229,281, Woo et al., filed Sep. 16, 2005.                                                                                                                                                                                                                                                      |
| U.S. Appl. No. 29/238,541, Braunschweig et al., filed Sep. 16, 2005.                                                                                                                                                                                                                                             |
| U.S. Appl. No. 29/238,542, Braunschweig et al., filed Sep. 16, 2005.                                                                                                                                                                                                                                             |
| U.S. Appl. No. 29/238,556, Braunschweig et al., filed Sep. 16, 2005.                                                                                                                                                                                                                                             |
| U.S. Appl. No. 29/246,256, Shimizu et al., filed Mar. 28, 2006.                                                                                                                                                                                                                                                  |
| U.S. Appl. No. 29/246,257, Shimizu et al., filed Mar. 28, 2006.                                                                                                                                                                                                                                                  |
| U.S. Appl. No. 29/246,258, Shimizu et al., filed Mar. 28, 2006.                                                                                                                                                                                                                                                  |
| U.S. Appl. No. 29/246,259, Shimizu et al., filed Mar. 28, 2006.                                                                                                                                                                                                                                                  |
| U.S. Appl. No. 29/246,260, Shimizu et al., filed Mar. 28, 2006.                                                                                                                                                                                                                                                  |
| U.S. Appl. No. 29/246,261, Shimizu et al., filed Mar. 28, 2006.                                                                                                                                                                                                                                                  |
| U.S. Appl. No. 29/253,148, Braunschweig et al., filed Feb. 1, 2006.                                                                                                                                                                                                                                              |
| U.S. Appl. No. 29/253,110, Braunschweig et al., filed Feb. 1, 2006.                                                                                                                                                                                                                                              |
| U.S. Appl. No. 29/253,085, Braunschweig et al., filed Feb. 1, 2006.                                                                                                                                                                                                                                              |
| U.S. Appl. No. 29/253,084, Braunschweig et al., filed Feb. 1, 2006.                                                                                                                                                                                                                                              |
| “robAust”, Roberlo Abrasives, Copyright © 2002-2006 robAust Pty Ltd., [retrieved from the internet on Jul. 6, 2006], URL < <a href="http://www.robaust.com/shopdisplayproducts.asp?id=30&amp;cat=Roberlo+Abrasives">http://www.robaust.com/shopdisplayproducts.asp?id=30&amp;cat=Roberlo+Abrasives</a> >, pp. 2. |

“List of Products”, Roberlo United States, © Copyright 2003 Roberloroberlousa.com, roberlo.com), [retrieved from the internet on Jan. 7, 2004], URL <<http://www.roberlousa.com/abrasives.htm>>, pp. 2.

\* cited by examiner



*Fig. 1*



*Fig. 2*



Fig. 3



Fig. 4





Fig. 6



*Fig. 7*



*Fig. 8*



*Fig. 9*

## 1

ABRASIVE ARTICLE AND METHODS OF  
MAKING SAME

## FIELD OF THE INVENTION

The present invention relates generally to an abrasive article and, more particularly, to a porous abrasive article that allows air and dust particles to pass through.

## BACKGROUND

Abrasive articles are used in industry for abrading, grinding, and polishing applications. They can be obtained in a variety of converted forms, such as belts, discs, sheets, and the like, in many different sizes.

Generally, when using abrasives articles in the form of "sheet goods" (i.e., discs and sheets), a back-up pad is used to mount or attach the abrasive article to the abrading tool. One method of attaching abrasive discs and sheets to back-up pads includes a two-part mechanical engagement system, such as, for example, a hook and loop fastener. When the attachment means is a hook and loop system, the abrasive article will have either a loop or the hook component on the backing surface opposite the abrasive coating, and the back-up pad will have the complementary mating component (i.e., a hook or loop).

One type of back-up pad has dust collection holes connected by a series of grooves to help control swarf build-up on the abrading surface of the abrasive article. The dust collection holes are typically connected to a vacuum source. The dust collection grooves and holes provide a passageway for removing particles such as swarf, dust, and debris from the abrading surface. The passageway can also be used to remove abrading fluids, such as water or oil, from the abrading surface.

In some configurations, particles and fluid pass from the abrading surface of the abrasive article to the back-up pad through holes cut in the abrasive article. The dust extraction capabilities of these designs are limited because of the intermittent presence of the holes. In other configurations, the abrasive article is made from a porous knitted cloth with integral loops, such as reported by Hoglund et al. in U.S. Pat. No. 6,024,634.

There is a continuing need for alternative ways to provide a cost effective abrasive article with a mechanical fastening system and dust extraction capabilities. It would be particularly desirable to provide a porous abrasive article in which the abrasive layer could be designed and manufactured independently of the attachment means.

## SUMMARY

The present invention relates generally to an abrasive article and, more particularly, to a porous abrasive article that allows air and dust particles to pass through.

In one aspect, the present invention provides an abrasive article with a screen abrasive comprising an open mesh backing having a first major surface that has a perimeter that defines a screen abrasive surface area, a second major surface, a plurality of openings extending from the first major surface to the second major surface, and an abrasive layer secured to at least a portion of the first major surface of the backing. The abrasive layer comprises a plurality of abrasive particles and at least one binder. An apertured attachment interface is associated with the second major surface of the open mesh backing. The apertured attachment interface comprises a base sheet that has a plurality of hooks

## 2

projecting from at least a portion of the base sheet, and a plurality of apertures extending through the base sheet. The apertures form a cumulative open area that is no greater than 40 percent of the screen abrasive surface area. The apertures cooperate with the screen abrasive to allow the flow of particles through the abrasive article.

In some embodiments, the abrasive article allows particles having a size of at least 10 micrometers to pass through the abrasive article.

10 In another aspect, the present invention provides a porous abrasive article. The abrasive article comprises a woven backing having a first major surface having a perimeter that defines a screen abrasive surface area, a second major surface, and a plurality of openings extending from the first major surface to the second major surface. An abrasive layer is secured to at least a portion of the first major surface of the backing. The abrasive layer comprises a plurality of abrasive particles and at least one binder. An apertured attachment interface is affixed to the second major surface of 15 the backing. The apertured attachment interface comprises a base sheet comprising a plurality of hooks projecting from at least a portion of the base sheet, and a plurality of apertures extending through the base sheet.

20 In some embodiments, the apertured attachment interface comprises a cumulative open area that is in the range of 5 to 30 percent of the screen abrasive surface area. In yet further embodiments, the apertured attachment interface comprises a cumulative open area that is in the range of 10 to 20 percent of the screen abrasive surface area.

25 In another aspect, the present invention provides methods for making abrasive articles having a screen abrasive and an apertured attachment interface that cooperates with the screen abrasive to allow the flow of particles through the abrasive article.

30 In another aspect, the present invention provides alternative ways to provide a cost effective abrasive article with a mechanical fastening system and dust extraction capabilities. The abrasive article is useful for abrading a variety of surfaces, including, for example, paint, primer, wood, plastic, fiberglass, and metal. In some embodiments, the abrasive layer can be designed and manufactured independently of the porous attachment interface, allowing the manufacturer to optimize the performance of the screen abrasive substantially independently of the selection of apertured attachment 35 interface, and vice versa.

40 The above summary of the present invention is not intended to describe each disclosed embodiment or every implementation of the present invention. The Figures and the detailed description that follow more particularly exemplify illustrative embodiments. The recitation of numerical ranges by endpoints includes all numbers subsumed with that range (e.g., 1 to 5 includes 1, 1.5, 2, 2.75, 3, 4, 4.80, and 5).

## 55 BRIEF DESCRIPTION OF THE DRAWING

FIG. 1 is a perspective view of an exemplary abrasive article according to the present invention partially cut away to reveal the apertured attachment interface;

60 FIG. 2 is a perspective view of an exemplary open mesh screen abrasive partially cut away to reveal the components of the abrasive layer;

65 FIG. 3 is a perspective view of an exemplary woven open mesh screen abrasive partially cut away to reveal the components of the abrasive layer;

FIG. 4 is a cross-sectional view of an exemplary abrasive article according to the present invention;

FIG. 5 is a SEM photomicrograph at 100 times of an abrasive surface of a screen abrasive article with abrasive particles that are not erectly oriented;

FIG. 6 is a SEM photomicrograph at 100 times of an abrasive surface of a screen abrasive of the present invention having erectly oriented abrasive particles;

FIG. 7 is a bottom view of an exemplary apertured attachment interface according to the present invention;

FIG. 8 is a bottom view of an exemplary apertured attachment interface according to the present invention; and

FIG. 9 is a bottom view of an exemplary apertured attachment interface according to the present invention with triangular apertures.

These figures, which are idealized, are not to scale and are intended to be merely illustrative of the present invention and non-limiting.

#### DETAILED DESCRIPTION

FIG. 1 shows a perspective view of an exemplary abrasive article 110 with a partial cut away. As shown in FIG. 1, the abrasive article 110 has a screen abrasive 112 on its upper surface and an apertured attachment interface 116 having a plurality of apertures 118 attached to the screen abrasive 112. The apertured attachment interface 116 cooperates with the screen abrasive 112 to allow the flow of particles through the abrasive article 110.

The apertured attachment interface forms the hook portion of a two-part mechanical engagement system.

Abrasive articles according to the present invention may be attached to a variety of surfaces having any suitable engaging structures, such as fibers, filaments (such as brushed nylon and brushed polyester), woven and nonwoven fabrics, knitted fabric, and stitch-bonded fabrics. Other applications are also contemplated, such as attachment to foam (particularly open-cell foam) or to a compatible set of engaging hooks. The apertured attachment interface is typically used to affix the abrasive article of the present invention to a back-up pad. The back-up pad typically includes a generally planar major surface with loops to which the apertured attachment interface of the abrasive article, such as a disc or sheet, may be attached.

Although back-up pads may be hand held, back-up pads are more commonly used in conjunction with a powered abrading apparatus such as electric or pneumatic sanders. The apertured attachment interface can be designed with hooks that permit the abrasive article to be removed from a back-up pad with a small amount of force. The hooks can also be designed to resist movement of the abrasive article relative to the loop faced back-up pad during use. The desired hook and loop dimensions will depend upon the shape and type of hooks provided and on the desired engagement characteristics of the abrasive article.

FIG. 2 is a perspective view of an exemplary open mesh screen abrasive 212 partially cut away to reveal the components of the abrasive layer. The screen abrasive 212 comprises an open mesh backing 222 covered with an abrasive layer. The open mesh backing 222 has a plurality of openings 224. The abrasive layer comprises a make coat 232, abrasive particles 230, and a size coat 234. A plurality of openings 214 extend through the screen abrasive 212.

The open mesh backing can be made from any porous material, including, for example, perforated films or woven or knitted fabrics. In the embodiment shown in FIG. 2, the open mesh backing 222 is a perforated film. The film for the backing can be made from metal, paper, or plastic, including molded thermoplastic materials and molded thermoset mate-

rials. In some embodiments, the open mesh backing is made from perforated or slit and stretched sheet materials. In some embodiments, the open mesh backing is made from fiberglass, nylon, polyester, polypropylene, or aluminum.

The openings 224 in the open mesh backing 222 can be generally square shaped as shown in FIG. 2. In other embodiments, the shape of the openings can be other geometric shapes, including, for example, a rectangle shape, a circle shape, an oval shape, a triangle shape, a parallelogram shape, a polygon shape, or a combination of these shapes. The openings 224 in the open mesh backing 222 can be uniformly sized and positioned as shown in FIG. 2. In other embodiments, the openings may be placed non-uniformly by, for example, using a random opening placement pattern, varying the size or shape of the openings, or any combination of random placement, random shapes, and random sizes.

FIG. 3 is a perspective view of an exemplary woven open mesh screen abrasive partially cut away to reveal the components of the abrasive layer. As shown in FIG. 3, the screen abrasive 312 comprises a woven open mesh backing 322 and an abrasive layer. The abrasive layer comprises a make coat 332, abrasive particles 330, and a size coat 334. A plurality of openings 314 extend through the screen abrasive 312.

The woven open mesh backing 322 comprises a plurality of generally parallel warp elements 338 that extend in a first direction and a plurality of generally parallel weft elements 336 that extend in a second direction. The weft 338 and warp elements 336 of the open mesh backing 322 form a plurality of openings 324. An optional lock layer 326 can be used to improve integrity of the open mesh backing or improve adhesion of the abrasive layer to the open mesh backing.

As shown in FIG. 3, the second direction is perpendicular to the first direction to form square shaped openings 324 in the woven open mesh backing 322. In some embodiments, the first and second directions intersect to form a diamond pattern. The shape of the openings can be other geometric shapes, including, for example, a rectangle shape, a circle shape, an oval shape, a triangle shape, a parallelogram shape, a polygon shape, or a combination of these shapes. In some embodiments, the warp and weft elements are yarns that are woven together in a one-over-one weave.

The warp and weft elements may be combined in any manner known to those in the art, including, for example, weaving, stitch-bonding, or adhesive bonding. The warp and weft elements may be fibers, filaments, threads, yarns or a combination thereof. The warp and weft elements may be made from a variety of materials known to those skilled in the art, including, for example, synthetic fibers, natural fibers, glass fibers, and metal. In some embodiments, the warp and weft elements comprise monofilaments of thermoplastic material or metal wire. In some embodiments, the woven open mesh backing comprises nylon, polyester, or polypropylene.

The openings 324 in the open mesh backing 322 can be uniformly sized and positioned as shown in FIG. 3. In other embodiments, the openings can be placed non-uniformly by, for example, using a random opening placement pattern, varying the size or shape of the openings, or any combination of random placement, random shapes, and random sizes.

The open mesh backing, whether woven or perforated, may comprise openings having different open areas. The "open area" of an opening in the mesh backing refers to the area of the opening as measured over the thickness of the mesh backing (i.e., the area bounded by the perimeter of material forming the opening through which a three-dimen-

sional object could pass). Open mesh backings useful in the present invention typically have an average open area of at least about 0.3 square millimeters per opening. In some embodiments, the open mesh backing has an average open area of at least about 0.5 square millimeters per opening. In yet further embodiments, the open mesh backing has an average open area of at least about 0.7 square millimeters per opening.

Typically, open mesh backings useful in the present invention have an average open area that is less than about 3.5 square millimeters per opening. In some embodiments, the open mesh backing has an average open area that is less than about 2.5 square millimeters per opening. In yet further embodiments, the open mesh backing has an average open area that is less than about 0.9 square millimeters per opening.

The open mesh backing, whether woven or perforated, comprises a total open area that affects the amount of air that can pass through the open mesh backing as well as the effective area and performance of the abrasive layer. The "total open area" of the mesh backing refers to the cumulative open areas of the openings as measured over a unit area of the mesh backing. Open mesh backings useful in the present invention have a total open area of at least about 0.5 square centimeters per square centimeter of backing (i.e., 50 percent open area). In some embodiments, the open mesh backing has a total open area of at least about 0.6 square centimeters per square centimeter of backing (i.e., 60 percent open area). In yet further embodiments, the open mesh backing has a total open area of at least about 0.75 square centimeters per square centimeter of backing (i.e., 75 percent open area).

Typically, open mesh backings useful in the present invention have a total open area that is less than about 0.95 square centimeters per square centimeter of backing (i.e., 95 percent open area). In some embodiments, the open mesh backing has a total open area that is less than about 0.9 square centimeters per square centimeter of backing (i.e., 90 percent open area). In yet further embodiments, the open mesh backing has a total open area that is less than about 0.82 square centimeters per square centimeter of backing (i.e., 82 percent open area).

FIG. 4 is a cross-sectional view of an exemplary abrasive article 410 according to the present invention. As shown in FIG. 4, the abrasive article 410 comprises a screen abrasive 412 affixed to an apertured attachment interface 416 having a plurality of apertures 418 using adhesive 440.

As shown in FIG. 4, the screen abrasive 412 comprises a woven open mesh backing 422 and an abrasive layer. The abrasive layer comprises a make coat 432, abrasive particles 430, and a size coat 434. The screen abrasive 412 comprises a plurality of generally parallel warp elements 438 that extend in a first direction and a plurality of generally parallel weft elements 436 that extend in a second direction. The weft 438 and warp elements 436 of the open mesh backing 422 form a plurality of openings.

The apertured attachment interface 416 comprises a plurality of hooks 420 integrally molded to a base sheet. As used herein, the term "hook" refers to a structure that enables the apertured attachment interface to releasably engage structures provided on an opposed surface. Hooks typically comprise a stem with a distal end that extends from the base sheet and a head proximate the distal end of the stem. The design of the hook may be selected from among numerous different designs known to those skilled in the art, including, for example, those reported in U.S. Pat. No. 6,579,161 (Chesley et al.) and U.S. Pat. No. 6,843,944 (Bay

et al.), which are incorporated herein by reference. It is understood that other hook designs are comprehended by the present invention, though they are not specifically described below.

5 The hooks, including the stem or head or any portion thereof, may have any suitable cross-sectional shape, taken parallel to the substrate, including but not limited to a circle, an oval, a polygon (such as a star, a cross, a rectangle, or a parallelogram), or a multi-lobed shape (such as a daisy or a clover). The hooks may be solid or hollow.

10 In some embodiments, the cross-sectional area of the stem of the hook taken parallel to the base sheet, is within the range of about 0.002 to 25 square millimeters. In other embodiments, the cross-sectional area of the stem of the hook taken parallel to the base sheet, is within the range of about 0.01 to 1 square millimeter. In yet further embodiments, the cross-sectional area of the stem of the hook taken parallel to the base sheet, is within the range of about 0.05 to 0.45 square millimeters.

15 In some embodiments, the overall height of the hook as measured perpendicular to the base sheet, is within the range of about 0.01 to 10 millimeters. In other embodiments, the overall height of the hook as measured perpendicular to the base sheet, is within the range of about 0.05 to 2.5 millimeters. In yet further embodiments, the overall height of the hook as measured perpendicular to the base sheet, is within the range of about 0.13 and 1 millimeter.

20 The shapes, diameters, and lengths of the plurality of hooks can be mixed within a given abrasive article, such that the abrasive article comprises hooks of more than one shape, diameter, and/or length. The shape, size, and orientation of the hooks may be selected to provide a suitable shear strength and peel strength for a given application.

25 The hooks may be straight, arcuate, or otherwise, and may be arranged in a regular array or be randomly distributed across the base sheet. For example, it may be desirable to provide a helical hook pattern, or to arrange the hooks in parallel, sinusoidal columns. The density of hooks can be selected as desired. In some embodiments, the density of hooks is between approximately 8 and 310 hooks per square centimeter, although other hook densities can be provided.

30 When the abrasive article is attached to an opposed surface, such as a surface having a plurality of loop members, not all of the hooks must engage with the structures 45 (such as a loop) of the opposed surface. Typically, a majority of the hooks will hook the structures of the engaging surface, and the disengagement force will typically be directly related to the number of hooks that are engaged. The percentage of hooks that are engaged by a particular opposed surface depends on many factors, such as hook dimensions and density, and the topography of the opposed surface.

35 The hooks may also be arranged in a plurality of clusters on the base sheet. That is, two or more hooks may be placed close to each other in a cluster, with adjacent clusters separated from each other by a distance greater than the distance between the hooks within a cluster. The hooks within each cluster could be inclined at any suitable orientation, although the hooks within each cluster can be inclined at different orientations. Furthermore, the clusters could be randomly or uniformly distributed over the surface to which the hooks are attached, as suitable to the particular application. Clusters can be provided in a plurality of rows, or stripes, and those rows may be parallel, including, for example, straight rows, or curvilinear rows.

40 The hook material can be an organic polymeric material, such as a thermosetting material or a thermoplastic material.

Useful materials include, but are not limited to, polyurethanes, polyamides, polyolefins (for example, polyethylene and polypropylene), polyesters, and combinations thereof. The hooks may also comprise one or more additives, including but not limited to fillers, fibers, antistatic agents, lubricants, wetting agents, surfactants, pigments, dyes, coupling agents, plasticizers, and suspending agents.

The material used to manufacture the apertured attachment interface of the present invention may be made in one of many different ways known to those skilled in the art. The hooks and base sheet can be formed integrally or formed independently. Several suitable processes for making fastener members useful in making apertured attachment interfaces used in the present invention, include, for example, methods described in U.S. Pat. No. 5,058,247 (Thomas et al.) (for low cost hook fasteners); U.S. Pat. No. 4,894,060 (Nestegard) (for diaper fasteners), U.S. Pat. No. 5,679,302 (Miller et al.) (entitled "Method for making a mushroom-type hook strip for a mechanical fastener"), and U.S. Pat. No. 6,579,161 (Chesley et al.), each of which is incorporated herein by reference.

Apertures can be formed in the base sheet using any methods known to those skilled in the art. For example, the apertures can be cut from a web of base sheet material with hooks using, for example, a die, laser, or other perforating instruments known to those skilled in the art. In other embodiments, the base sheet can be formed with apertures.

The screen abrasive 412 may be adhered to the apertured attachment interface 416 using any suitable form of attachment, such as, for example, glue, pressure sensitive adhesive, hot-melt adhesive, spray adhesive, thermal bonding, and ultrasonic bonding.

The screen abrasive is affixed to the apertured attachment interface in a manner that does not prevent the flow of particles through the abrasive article. In some embodiments, the screen abrasive is adhered to the apertured attachment interface in a manner that does not substantially inhibit the flow of particles through the abrasive article. The level of particle flow through the abrasive article can be restricted, at least in part, by the introduction of an adhesive between the screen abrasive and the apertured attachment interface. The level of restriction can be minimized by applying the adhesive to the screen abrasive in a discontinuous fashion such as, for example, as discrete adhesive areas (e.g., atomized spray or starved extrusion die) or distinct adhesive lines (e.g., hot melt swirl-spray or patterned roll coater).

In some embodiments, the particles of swarf, dust, or debris that can flow through the abrasive article of the present invention have a particle size of at least 10 micrometers. In some embodiments, at least 30 micrometer particles can pass through the abrasive article. In yet further embodiments, at least 45 micrometer particles can pass through the abrasive article.

In some embodiments, the screen abrasive is adhered to the apertured attachment interface by applying a spray adhesive, such as, for example, "3M BRAND SUPER 77 ADHESIVE", available from 3M Company, St. Paul, Minn., to one side of the screen abrasive. In other embodiments, a hot-melt adhesive is applied to one side of the screen abrasive using either a hot-melt spray gun or an extruder with a comb-type shim. In yet further embodiments, a preformed adhesive porous mesh is placed between the screen abrasive and the apertured attachment interface.

Adhesives useful in the present invention include both pressure sensitive and non-pressure sensitive adhesives. Pressure sensitive adhesives are normally tacky at room temperature and can be adhered to a surface by application

of, at most, light finger pressure, while non-pressure sensitive adhesives include solvent, heat, or radiation activated adhesive systems. Examples of adhesives useful in the present invention include those based on general compositions of polyacrylate; polyvinyl ether; diene-containing rubbers such as natural rubber, polyisoprene, and polyisobutylene; polychloroprene; butyl rubber; butadiene-acrylonitrile polymers; thermoplastic elastomers; block copolymers such as styrene-isoprene and styrene-isoprene-styrene block copolymers, ethylene-propylene-diene polymers, and styrene-butadiene polymers; polyalphaolefins; amorphous polyolefins; silicone; ethylene-containing copolymers such as ethylene vinyl acetate, ethylacrylate, and ethylmethacrylate; polyurethanes; polyamides; polyesters; epoxies; polyvinylpyrrolidone and vinylpyrrolidone copolymers; and mixtures of the above. Additionally, the adhesives can contain additives such as tackifiers, plasticizers, fillers, antioxidants, stabilizers, pigments, diffusing particles, curatives, and solvents.

As discussed above, the abrasive layer of the screen abrasive comprises a plurality of abrasive particles and at least one binder. In some embodiments, the abrasive layer comprises a make coat, a size coat, a supersize coat, or a combination thereof. In some embodiments, a treatment can be applied to the open mesh backing such as, for example, a presize, a backsize, a subsize, or a saturant.

Typically, the make layer of a coated abrasive is prepared by coating at least a portion of the open mesh backing (treated or untreated) with a make layer precursor. Abrasive particles are then at least partially embedded (e.g., by electrostatic coating) to the make layer precursor comprising a first binder precursor, and the make layer precursor is at least partially cured. Electrostatic coating of the abrasive particles typically provides erectly oriented abrasive particles. In the context of the present invention, the term "erectly oriented" refers to a characteristic in which the longer dimensions of a majority of the abrasive particles are oriented substantially perpendicular (i.e., between 60 and 120 degrees) to the backing. Other techniques for erectly orienting abrasive particles can also be used.

FIG. 6 is a SEM photomicrograph at 100 times of an abrasive surface of a screen abrasive of the present invention having erectly oriented abrasive particles. FIG. 5 is a SEM photomicrograph at 100 times of an abrasive surface of a screen abrasive article with abrasive particles that are not erectly oriented.

Next, the size layer is prepared by coating at least a portion of the make layer and abrasive particles with a size layer precursor comprising a second binder precursor (which may be the same as, or different from, the first binder precursor), and at least partially curing the size layer precursor. In some coated abrasive articles, a supersize is applied to at least a portion of the size layer. If present, the supersize layer typically includes grinding aids and/or anti-loading materials.

Typically, a binder is formed by curing (e.g., by thermal means, or by using electromagnetic or particulate radiation) a binder precursor. Useful first and second binder precursors are known in the abrasive art and include, for example, free-radically polymerizable monomer and/or oligomer, epoxy resins, acrylic resins, urethane resins, phenolic resins, urea-formaldehyde resins, melamine-formaldehyde resins, aminoplast resins, cyanate resins, or combinations thereof. Useful binder precursors include thermally curable resins and radiation curable resins, which may be cured, for example, thermally and/or by exposure to radiation.

Suitable abrasive particles for the screen abrasive that can be used in the abrasive article of the present invention can be any known abrasive particles or materials commonly used in abrasive articles. Examples of useful abrasive particles for coated abrasives include, for example, fused aluminum oxide, heat treated aluminum oxide, white fused aluminum oxide, black silicon carbide, green silicon carbide, titanium diboride, boron carbide, tungsten carbide, titanium carbide, diamond, cubic boron nitride, garnet, fused alumina zirconia, sol gel abrasive particles, silica, iron oxide, chromia, ceria, zirconia, titania, silicates, metal carbonates (such as calcium carbonate (e.g., chalk, calcite, marl, travertine, marble and limestone), calcium magnesium carbonate, sodium carbonate, magnesium carbonate), silica (e.g., quartz, glass beads, glass bubbles and glass fibers) silicates (e.g., talc, clays, (montmorillonite) feldspar, mica, calcium silicate, calcium metasilicate, sodium aluminosilicate, sodium silicate) metal sulfates (e.g., calcium sulfate, barium sulfate, sodium sulfate, aluminum sodium sulfate, aluminum sulfate), gypsum, aluminum trihydrate, graphite, metal oxides (e.g., tin oxide, calcium oxide), aluminum oxide, titanium dioxide) and metal sulfites (e.g., calcium sulfite), metal particles (e.g., tin, lead, copper), plastic abrasive particles formed from a thermoplastic material (e.g., polycarbonate, polyetherimide, polyester, polyethylene, polysulfone, polystyrene, acrylonitrile-butadiene-styrene block copolymer, polypropylene, acetal polymers, polyvinyl chloride, polyurethanes, nylon), plastic abrasive particles formed from crosslinked polymers (e.g., phenolic resins, aminoplast resins, urethane resins, epoxy resins, melamine-formaldehyde, acrylate resins, acrylated isocyanurate resins, urea-formaldehyde resins, isocyanurate resins, acrylated urethane resins, acrylated epoxy resins), and combinations thereof. The abrasive particles may also be agglomerates or composites that include additional components, such as, for example, a binder. Criteria used in selecting abrasive particles used for a particular abrading application typically include: abrading life, rate of cut, substrate surface finish, grinding efficiency, and product cost.

Coated screen abrasives can further comprise optional additives, such as, abrasive particle surface modification additives, coupling agents, plasticizers, fillers, expanding agents, fibers, antistatic agents, initiators, suspending agents, photosensitizers, lubricants, wetting agents, surfactants, pigments, dyes, UV stabilizers, and suspending agents. The amounts of these materials are selected to provide the properties desired. Additives may also be incorporated into the binder, applied as a separate coating, held within the pores of the agglomerate, or combinations of the above.

Coated screen abrasive articles may be converted, for example, into belts, rolls, discs (including perforated discs), and/or sheets. One form of a coated screen abrasive useful in finishing operations is a disc. Abrasive discs are often used for the maintenance and repair of automotive bodies and wood finishing. The discs can be configured for use with a variety of tools, including, for example, electric or air grinders. The tool used to support the disc can have a self-contained vacuum system or can be connected to a vacuum line to help contain dust.

FIGS. 7-9 show bottom view of three exemplary apertured attachment interfaces with various aperture configurations. As shown in FIG. 7, the apertured attachment interface 716 has a plurality of hooks 720 and a plurality of apertures 718. The apertures 718 are circular and are configured in a pattern that is centered proximate the center of

the apertured attachment interface 716 such that no apertures are interrupted by the perimeter of the apertured attachment interface 716.

As shown in FIG. 8, the apertured attachment interface 816 has a plurality of hooks 820 and a plurality of apertures 818. The apertures 818 are circular and are configured in a pattern that is positioned randomly relative to the attachment interface 816 such that some apertures are interrupted by the perimeter of the apertured attachment interface 816.

As shown in FIG. 9, the apertured attachment interface 916 has a plurality of hooks 920 and a plurality of apertures 918. The apertures 918 are triangular and are configured in a pattern that is centered proximate the center of the apertured attachment interface 916 such that no apertures are interrupted by the perimeter of the apertured attachment interface 916.

Other shapes and geometries of apertures can also be used, including, for example, squares, ovals, stars, and polygons. The apertures can be of a uniform shape and size or vary in size or shape. In some embodiments, the vacuum port configuration of the back-up pad is considered when selecting the shape, size, and placement of the apertures in the attachment interface.

Typically, apertures useful in the present invention have an average open area no greater than 20 square millimeters per aperture. In some embodiments, the average open area is no greater than 15 square millimeters per aperture. In some embodiments, the average open area is no greater than 10 square millimeters per aperture. In yet further embodiments, the average open area is no greater than 8 square millimeters per aperture

Typically, apertures useful in the present invention have an average open area of at least 0.1 square millimeters per aperture. In some embodiments, the average open area is at least 0.5 square millimeters per aperture. In some embodiments, the average open area is at least 1 square millimeter per aperture. In yet further embodiments, the average open area is at least 2 square millimeters per aperture.

The apertured attachment interface comprises a cumulative open area that affects the amount of air and particles that can pass through the apertured attachment interface as well as the effective support area for the screen abrasive and, therefore, the performance of the abrasive layer. The "cumulative open area" of the apertured attachment interface refers to the sum of the open areas of the openings as measured over the screen abrasive surface area. The term "screen abrasive surface area" refers to the total area formed by the perimeter of the screen abrasive without consideration of any open areas in the screen. For example, an abrasive article comprising a screen abrasive with a 10 centimeter outer diameter having an apertured attachment interface with 20 apertures, each having an open area of 1 square centimeter, would have a cumulative open area of 0.25 square centimeters per square centimeter of screen abrasive (i.e., 25 percent cumulative open area).

Apertured attachment interfaces useful in the present invention have a cumulative open area no greater than 0.4 square centimeters per square centimeter of screen abrasive (i.e., 40 percent cumulative open area). In some embodiments, the apertured attachment interface has a cumulative open area no greater than 0.3 square centimeters per square centimeter of screen abrasive (i.e., 30 percent cumulative open area). In yet further embodiments, the apertured attachment interface has a cumulative open area no greater than 0.2 square centimeters per square centimeter of screen abrasive (i.e., 20 percent cumulative open area).

## 11

Typically, apertured attachment interfaces useful in the present invention have a total open area that is at least 0.02 square centimeters per square centimeter of screen abrasive (i.e., 2 percent cumulative open area). In some embodiments, the apertured attachment interface has a total open area that is at least 0.05 square centimeters per square centimeter of screen abrasive (i.e., 5 percent cumulative open area). In yet further embodiments, the apertured attachment interface has a total open area that is at least 0.10 square centimeters per square centimeter of screen abrasive (i.e., 10 percent cumulative open area).

Porosity for the abrasive article of the present invention can be measured with a Gurley Densitometer Model 4410. The Gurley Densitometer measures the amount of time, in seconds, required for 300 cubic centimeters of air to pass through a 0.65 square centimeter area of the abrasive article using a 1.39 Joules per meter force. The Gurley apparatus and procedures for its use are known in the textile industry. For purposes of the present invention, an abrasive article shall be considered "porous" if it has a Gurley porosity that is less than 5 seconds per 300 cubic centimeters of air for at least one 0.65 square centimeter area of the abrasive article.

In some embodiments, the abrasive article of the present invention has a Gurley porosity that is no greater than 5 seconds per 300 cubic centimeters of air. In other embodiments, the abrasive article of the present invention has a Gurley porosity that is no greater than 1.5 seconds per 300 cubic centimeters of air. In yet further embodiments, the abrasive article has a Gurley porosity that is no greater than 1 second per 300 cubic centimeters of air.

Advantages and other embodiments of this invention are further illustrated by the following examples, but the particular materials and amounts thereof recited in these examples, as well as other conditions and details, should not be construed to unduly limit this invention. For example, the basis weight, thickness, and composition of the apertured attachment interface can vary. All parts and percentages are by weight unless otherwise indicated.

Unless otherwise noted, all parts, percentages, and ratios reported in the following examples are on a weight basis, and all reagents used in the examples were obtained, or are available, from general chemical suppliers such as the Sigma-Aldrich Chemical Company, Saint Louis, Mo., or may be synthesized by conventional techniques.

## EXAMPLES

## Sanding Test #1

Using a razor blade, interconnecting U-shaped channels, 0.95 centimeter wide by 0.64 centimeter deep, were carved between the five holes of a 12.7 centimeter diameter by 1.6 centimeter thick foam back up pad, available under the trade designation "3M HOOKIT II BACKUP PAD, PART NUMBER 05345" from 3M Company, St. Paul, Minn. A 12.7 centimeter diameter sample disc was attached to the back up pad and then the pad mounted onto a fine finishing dual-action orbital sander, model "21034" from Dynabrade Corporation, Clarence, N.Y. A central dust extraction vacuum line was then attached to the sander. The abrasive layer was manually brought into contact with a pre-weighed 38.1 centimeter by 53.3 centimeter acrylic test panel, obtained from Seelye-Eiler Plastics Inc., Bloomington, Minn. The sander was run at 88.5 pounds per square inch (610.2 kilopascals) air line pressure and a down force of 12 pounds (5.4 kilograms) for 45 seconds. An angle of zero degrees to the surface of the workpiece was used. The 45 second

## 12

abrading cycle was repeated another 4 times, for a total of 3 minutes and 45 seconds. After the final sanding cycle the test panel was re-weighed and the sanding procedure repeated two more times, from which the average cut was determined. A visual observation of swarf on the abrasive surface was also made at the completion of the sanding test.

## Sanding Test #2

A 12.7 centimeter diameter sample disc was attached to a 12.7 centimeter by 1.6 centimeter thick foam back up pad, available under the trade designation "3M HOOKIT II BACKUP PAD, PART NUMBER 05245" from 3M Company. The back up pad was then mounted onto the model "21034" sander and, with the central dust extraction vacuum line disconnected, the sanding protocol as described in sanding test #1 was replicated.

## Sanding Test #3

A 45.7 centimeter by 76.2 centimeter mild steel test panel, was coated with a black primer, commercially available under the trade designation "SIKKENS COLORBUILD BLACK" from Akzo Nobel Coatings, Inc., Norcross, Ga., and allowed to cure at least 24 hours at 20 degrees Celsius. Using a razor blade, interconnecting U-shaped channels, 0.95 centimeter (cm) wide by 0.64 centimeter deep, were carved between the five holes of a 12.7 centimeter diameter by 1.6 centimeter thick foam back up pad, available under the trade designation "3M HOOKIT II BACKUP PAD, PART NUMBER 05345" from 3M Company. A 12.7 centimeter diameter sample disc was attached to the back up pad and then the pad mounted onto the model "21034" sander.

A central dust extraction vacuum line was then attached to the sander. The abrasive layer was manually brought into contact with the test panel and the sander run at 88.5 pounds per square inch (610.2 kilopascals) air line pressure, and a down force of 12 pounds (5.4 kilograms), for 30 seconds. An angle of 2.5 degrees to the surface of the workpiece was used. The 30 second abrading cycle is repeated another 5 times, wherein the 1<sup>st</sup>, 2<sup>nd</sup> and 6<sup>th</sup> cycles were run on unsanded primer and the 3<sup>rd</sup>, 4<sup>th</sup> and 5<sup>th</sup> cycles were run on the sanded primer area. After the final sanding cycle the test panel was re-weighed and the sanding procedure repeated two more times, from which the average cut was determined. A visual observation of swarf on the abrasive surface was also made at the completion of the sanding test.

## Sanding Test #4

A 15.2 centimeter diameter piece of loop fabric was applied to the face of a pressure sensitive adhesive (PSA) foam back up pad, available under the trade designation "3M STIKIT BACKUP PAD, PART NUMBER 05575" from 3M Company. A 15.2 centimeter diameter sample disc was then attached to the back up pad and the pad mounted onto a model "21039" sander from Dynabrade Corporation. The central dust extraction vacuum line disconnected and the sanding protocol as described in sanding test #3 was replicated. A visual observation of swarf on the test panel was also made at the completion of the sanding test.

## Sanding Test #5

A 55.8 centimeter by 81.3 centimeter mild steel test panel, primed with "URO1140S", from Dupont Automotive, Inc., Detroit, Mich., and subsequently pre-sanded, was used for the following test. A 12.7 centimeter diameter sample disc was attached to the back up pad described in Sanding Test #1. The pad was then mounted onto the model "21034" sander and a central dust extraction vacuum line attached to the sander. The abrasive layer was manually brought into contact with the pre-sanded test panel. The sander was run

at 90 pounds per square inch (620.5 kilopascals) air line pressure and a down force of 12 pounds (5.4 kilograms) for 30 seconds. An angle of zero degrees to the surface of the workpiece was used. The 60 second abrading cycle is repeated another 3 times, for a total of 4 minutes, from which the total average cut per sample was determined and the weight of swarf collected in the dust bag recorded.

#### Screen Abrasive

A screen abrasive was prepared as follows. A phenolic resin, available under the trade designation "BAKELITE PHENOLIC RESIN" from Bakelite Epoxy Polymer Corporation, Augusta, Ga., was dispersed to 56 percent solids in a 90:10 by weight water:polysolve medium, then diluted to 35 percent by weight solids with ethanol. The resin dispersion was applied as a make coat to a fiberglass plain weave screen, available under the trade designation "1620-12" from Hexcel Reinforcements, Anderson, S.C. Grade P320 alumina abrasive mineral, obtained under the trade designation "FSX" from Triebacher Schleifmittel AG, Villach, Austria was electrostatic ally coated onto the resin, cured for 2 hours at 205 degrees Fahrenheit (96 degrees Celsius). An aqueous size coat, 35 percent by weight phenolic resin, was then applied over the make coat and mineral, and the coating cured for 16 hours at 212 degrees Fahrenheit (100 degrees Celsius). A 30 percent by weight aqueous dispersion of 85:15 by weight zinc stearate polyacrylate was then applied over the size coat and dried at 180 degrees Fahrenheit (82.2 degrees Celsius)) for 15 minutes.

#### Attachment Interface 1 (AB1)

The hook component of a releasable mechanical fastener system was made according to the method described in U.S. Pat. No. 6,843,944 (Bay et al.), incorporated herein by reference. The resultant polypropylene attachment interface, had a 5 mils (127 micrometers) thickness, stem diameter 14 mils (355.6 micrometers), cap diameter 30 mils (0.76 millimeters), stem height 20 mils (508 micrometers) and a frequency of 340 stems per square inch (52.7 stems per square centimeter). The backing was not perforated.

#### Attachment Interface 2 (AB2)

The polypropylene attachment interface AB1 was uniformly perforated with a series of apertures,  $\frac{1}{16}^{\text{th}}$  inch (1.59 millimeters) diameter, using a 10.6 micrometer wavelength CO<sub>2</sub> laser, from Coherent, Inc., Santa Clara, Calif. The perforation frequency was 2.19 apertures per square centimeter, resulting in a backing having a cumulative open area of 5 percent.

#### Attachment Interface 3 (AB3)

The polypropylene attachment interface AB1 was uniformly perforated with a series of apertures,  $\frac{3}{32}^{\text{th}}$  inch (2.38 millimeters) diameter, according to the method described in AB2. The perforation frequency was 2.19 apertures per square centimeter, resulting in a backing having an open area of 11 percent.

#### Attachment Interface 4 (AB4)

The polypropylene attachment interface AB1 was uniformly perforated with a series of apertures,  $\frac{7}{64}^{\text{th}}$  inch (2.78 millimeters) diameter, according to the method described in AB2. The perforation frequency was 2.19 apertures per square centimeter, resulting in a backing having an open area of 15 percent.

#### Attachment Interface 5 (AB5)

The polypropylene attachment interface AB1 was uniformly perforated with a series of apertures,  $\frac{1}{8}^{\text{th}}$ -inch (3.18 millimeters) diameter, according to the method described in

AB2. The perforation frequency was 2.19 apertures per square centimeter, resulting in a backing having an open area of 20 percent.

#### Comparative A

An adhesive, type "3M 77 SPRAY ADHESIVE" from 3M Company, was lightly sprayed onto the non-abrasive side of the screen abrasive and to one side of AB1, and the two materials laminated together. 12.7 centimeter discs were then die cut from the laminate sheet.

#### Comparative B

A 5-inch (12.7 centimeter) grade P320 alumina abrasive film disc, commercially available under the trade designation "HOOKIT II P320 334U" from 3M Company.

#### Example 1

The non-abrasive side of screen abrasive was laminated to one side of AB2 according to the method described in Comparative A. Likewise, 12.7 centimeter sample discs were then die cut from the laminate.

#### Example 2

The non-abrasive side of screen abrasive was laminated to one side of AB3 according to the method described in Comparative A. Likewise, 12.7 centimeter sample discs were then die cut from the laminate.

#### Example 3

The non-abrasive side of screen abrasive was laminated to one side of AB4 according to the method described in Comparative A. Likewise, 12.7 centimeter sample discs were then die cut from the laminate.

#### Example 4

The non-abrasive side of screen abrasive was laminated to one side of AB5 according to the method described in Comparative A. Likewise, 12.7 centimeter sample discs were then die cut from the laminate.

#### Example 5

An adhesive, type "3M 77 SPRAY ADHESIVE" from 3M Company, was lightly sprayed onto the non-abrasive side of the screen abrasive and to one side of AB1, and the two materials laminated together. The laminate was then uniformly perforated with a series of apertures,  $\frac{1}{8}^{\text{th}}$ -inch (3.18 millimeters) diameter, according to the method described in AB2. The perforation frequency was 2.19 apertures per square centimeter, resulting in a backing having a cumulative open area of 20 percent. 12.7 centimeter discs were then die cut from the laminate sheet.

Comparative A and Example 4 were subjected to Sanding Test 1. Results are listed in Table 1.

TABLE 1

| Sample        | Average Total Cut (grams) | Swarf Present on Abrasive Surface |
|---------------|---------------------------|-----------------------------------|
| Comparative A | 4.8                       | Yes                               |
| Example 4     | 6.4                       | No                                |

Comparative A and Examples 2-4 were subjected to Sanding Test 2. Results are listed in Table 2.

TABLE 2

| Sample        | Average Total Cut (grams) | Swarf Present on Abrasive Surface | 5 |
|---------------|---------------------------|-----------------------------------|---|
| Comparative A | 3.8                       | Yes                               |   |
| Example 2     | 5.7                       | No                                |   |
| Example 3     | 7.2                       | No                                |   |
| Example 4     | 6.4                       | No                                |   |

Comparative A and Examples 1–4 were subjected to Sanding Test 3. Results are listed in Table 3.

TABLE 3

| Sample        | Average Total Cut (grams) | Swarf Present on Abrasive Surface | 15 |
|---------------|---------------------------|-----------------------------------|----|
| Comparative B | 7.9                       | Yes                               |    |
| Example 1     | 8.7                       | No                                |    |
| Example 2     | 9.2                       | No                                |    |
| Example 3     | 8.7                       | No                                |    |
| Example 4     | 8.8                       | No                                |    |

Comparative A and Examples 1–5 were subjected to Sanding Test 4. Results are listed in Table 4.

TABLE 4

| Sample        | Average Total Cut (grams) | Swarf Present on Test Panel | 30 |
|---------------|---------------------------|-----------------------------|----|
| Comparative A | 12.8                      | Yes                         |    |
| Example 1     | 12.9                      | Yes                         |    |
| Example 2     | 14.3                      | Yes                         |    |
| Example 3     | 14.0                      | No                          |    |
| Example 4     | 13.7                      | No                          |    |
| Example 5     | 12.1                      | No                          |    |

Comparative A and Example 4 were subjected to Sanding Test #5. Results are listed in Table 5.

TABLE 5

| Sample        | Average Total Cut (grams) | Swarf Collected (grams) | 40 |
|---------------|---------------------------|-------------------------|----|
| Comparative A | 16.6                      | 1.4                     |    |
| Example 4     | 23.6                      | 15.8                    |    |

It is to be understood that even in the numerous characteristics and advantages of the present invention set forth in above description and examples, together with details of the structure and function of the invention, the disclosure is illustrative only. Changes can be made to detail, especially in matters of the dimensions and compositions of the screen abrasive and apertured attachment interface within the principles of the invention to the full extent indicated by the meaning of the terms in which the appended claims are expressed and the equivalents of those structures and methods.

What is claimed is:

1. An abrasive article comprising:

a screen abrasive comprising an open mesh backing having a first major surface having a perimeter that defines a screen abrasive surface area, a second major surface, a plurality of openings extending from said first major surface to said second major surface, and an abrasive layer secured to at least a portion of said first

major surface of said backing, said abrasive layer comprising a plurality of abrasive particles and at least one binder; and

an apertured attachment interface adhered to said second major surface of said open mesh backing, said apertured attachment interface comprising a base sheet comprising a plurality of hooks projecting from at least a portion of said base sheet, and a plurality of apertures extending through said base sheet, said apertures forming a cumulative open area that is no greater than 40 percent of said screen abrasive surface area, wherein said apertures cooperate with said screen abrasive to allow the flow of particles through said abrasive article.

2. The abrasive article of claim 1 wherein said open mesh backing is woven.

3. The abrasive article of claim 2 wherein said open mesh backing comprises at least one of fiberglass, nylon, polyester, polypropylene, or aluminum.

4. The abrasive article of claim 1 wherein said open mesh backing is a perforated film.

5. The abrasive article of claim 1 wherein said openings in said open mesh backing have an average open area of at least 0.3 square millimeters.

6. The abrasive article of claim 1 wherein said openings in said open mesh backing have a total open area of at least 50 percent of said screen abrasive surface area.

7. The abrasive article of claim 1 wherein said particles that flow through said abrasive article comprise particles having a size of at least 10 micrometers.

8. The abrasive article of claim 1 wherein said apertures are circular.

9. The abrasive article of claim 1 wherein said apertures have an average open area in the range of 0.5 to 8 square millimeters per aperture.

10. The abrasive article of claim 1 wherein said apertures form a cumulative open area that is in the range of 5 to 30 percent of said screen abrasive surface area.

11. The abrasive article of claim 1 wherein said apertures form a cumulative open area that is in the range of 10 to 20 percent of said screen abrasive surface area.

12. The abrasive article of claim 1 wherein said plurality of hooks comprise a polymeric material selected from a polyurethane, polyamide, polyolefin, polyester, or combinations thereof.

13. The abrasive article of claim 1 wherein said plurality of hooks comprise a polymeric material selected from at least one of polyethylene or polypropylene.

14. The abrasive article of claim 1 further comprising adhesive securing said apertured attachment interface to said second major surface of said open mesh backing.

15. The abrasive article of claim 1 wherein said abrasive particles are erectly oriented.

16. An abrasive article comprising:  
a woven backing having a first major surface having a perimeter that defines a screen abrasive surface area, a second major surface, and a plurality of openings extending from said first major surface to said second major surface;

an abrasive layer secured to at least a portion of said first major surface of said backing, said abrasive layer comprising a plurality of abrasive particles and at least one binder; and

an apertured attachment interface affixed to said second major surface of said backing, said apertured attachment interface comprising a base sheet comprising a

**17**

plurality of hooks projecting from at least a portion of said base sheet, and a plurality of apertures extending through said base sheet,

wherein said abrasive article is porous.

**17.** The abrasive article of claim **16** wherein said apertured attachment interface comprises a cumulative open area that is in the range of 5 to 30 percent of said screen abrasive surface area. 5

**18.** The abrasive article of claim **16** wherein said apertured attachment interface comprises a cumulative open area that is in the range of 10 to 20 percent of said screen abrasive surface area. 10

**19.** The abrasive article of claim **16** wherein said apertures have an average open area in the range of 0.5 to 8 square millimeters per aperture. 15

**20.** A method of making an abrasive article comprising: providing a screen abrasive comprising an open mesh backing having a first major surface having a perimeter that defines a screen abrasive surface area, a second

**18**

major surface, a plurality of openings extending from said first major surface to said second major surface, and an abrasive layer affixed to at least a portion of said first major surface of said backing, said abrasive layer comprising a plurality of abrasive particles and at least one binder;

providing an attachment interface comprising a base sheet comprising a plurality of hooks projecting from at least a portion of said base sheet;

perforating said attachment interface to form an apertured attachment interface comprising a plurality of apertures extending through said base sheet, said apertures forming a cumulative open area that is no greater than 40 percent of said screen abrasive surface area; and affixing said apertured attachment interface to at least a portion of said second major surface of said open mesh backing.

\* \* \* \* \*

UNITED STATES PATENT AND TRADEMARK OFFICE  
**CERTIFICATE OF CORRECTION**

PATENT NO. : 7,252,694 B2  
APPLICATION NO. : 11/198,265  
DATED : August 7, 2007  
INVENTOR(S) : Edward J. Woo

Page 1 of 1

It is certified that error appears in the above-identified patent and that said Letters Patent is hereby corrected as shown below:

Column 3

Line 42, after "attached" insert -- . --.

Column 6

Line 65, delete "curvilinear" and insert -- curvilinear -- therefor.

Column 8

Line 62, delete "resings," and insert -- resins -- therefor.

Column 10

Line 32, after "aperture" insert -- . --.

Column 16

Line 10, in Claim 1, delete "then" and insert -- than -- therefor.

Column 18

Line 13, in Claim 20, delete "then" and insert -- than -- therefor.

Signed and Sealed this

Fifteenth Day of April, 2008



JON W. DUDAS  
*Director of the United States Patent and Trademark Office*